# EUROPEAN PATENT SPECIFICATION

(11) **EP 1 789 521 B1**
(45) Date of publication and mention of the grant of the patent: **01.05.2013**
(21) Application number: 05756861.0
(22) Date of filing: 07.07.2005
(51) Int. Cl.: C10M 163/00, C10M 167/00, C10M 169/04

(54) **LUBRICATING OIL COMPOSITION**
SCHMIERÖLZUSAMMENSETZUNG
COMPOSITION D'HUILE LUBRIFIANTE

(30) Priority: 09.07.2004 EP 04016206
(43) Date of publication of application: 30.05.2007
(73) Proprietor: Shell Internationale Research Maatschappij B.V., 2596 HR Den Haag (NL)
(72) Inventor: BUSSE, Peter, 21107 Hamburg (DE); LEONHARDT, Helmut, 21107 Hamburg (DE); SANT, Peter, London SE1 7NA (GB); WILLARS, Malcolm, J., P.O. Box 1 Chester Cheshire CH1 3SH (GB)
(74) Representative: Matthezing, Robert Maarten
(86) International application number: PCT/EP2005/053241
(87) International publication number: WO 2006/005713

(56) References cited:
- EP-A- 1 104 800
- EP-A- 1 167 497
- WO-A-03/099972
- US-A1- 2003 148 900
- US-A1- 2004 102 335

## Description

The present invention relates to the use of a lubricating oil composition, in particular of a lubricating oil composition which is suitable for lubricating internal combustion engines.

Total Base Number (TBN) is a measure of how well a lubricating oil composition can neutralise acidic by-products of combustion/oxidation and is defined as the quantity of acid, expressed in terms of the equivalent number of milligrams of potassium hydroxide, that is required to neutralize all basic constituents present in 1 gram of a sample of the lubricating oil composition (test methods include, for example, ISO 3771, ASTM D-2896 and ASTM D-4739).

A high TBN is desirable in lubricating oil compositions in order to control corrosive engine wear from the acidic by-products of combustion/oxidation. Detergent additives in a lubricating oil composition are the primary source of alkalinity (TBN) and help to control, for example, top-ring deposits and bore polish.

Hence, metal-based detergents are the primary source of TBN in crankcase lubricating oil compositions.

In view of the adverse affects that the sulphated ash, sulphur and phosphorus concentrations of lubricating oil compositions may have on vehicle exhaust after-treatment devices, there is a trend towards lubricating oil compositions having reduced sulphated ash, sulphur and/or phosphorus concentrations therein (i.e. so-called low-SAPS lubricating oil compositions).

Phosphorus concentrations may be generally seduced by reducing the amount of zinc dithiophosphates which are present as anti-wear additives in lubricating oil compositions.

Sulphur levels in lubricating oil compositions may be reduced by employing low sulphur level base oils and reducing the amount of sulphur-containing additives employed therein.

Sulphated ash is the total weight percent of residue remaining after a lubricating oil composition has been carbonised, and the residue subsequently treated with sulphuric acid and heated to constant weight. The sulphated ash content in a lubricating oil composition is related to the total metal content therein. Sulphated ash may be conveniently measured according to ASTM D874.

The major sources of sulphated ash in a lubricating oil composition are generally any metal detergent additives and zinc dithiophosphate anti-wear additives that are employed therein.

Hence, in current low-SAPS lubricating oil compositions, sulphated ash levels, and consequently detergent levels, are low. As a result, the starting TBN (i.e. of fresh un-used lubricating oil compositions) of low-SAPS lubricating oil compositions tends to be lower than in lubricating oil compositions having higher sulphated ash, sulphur and/or phosphorus concentrations therein.

Thus, TBN retention (i.e. the ability to maintain an advantageous TBN level throughout the lifetime of a lubricating oil composition) is of increased importance for low-SAPS lubricating oil compositions which have lower starting TBNs.

US 2004/0102335 A1 describes lubricating oil compositions containing an additive formulation including at least one sulphonate, saligenin and salixarate detergent.

However, it is apparent from the Working Examples in US 2004/0102335 A1 that said lubricating oil compositions employ high TBN detergents therein.

In this regard, it is of note that the Working Examples in US 2004/0102335 A1 all employ a high TBN calcium sulphonate detergent therein as a TBN booster.

Furthermore, US 2004/0102335 A1 is concerned with the development of lubricating oil compositions with improved wear performance and is not directed to the problem of TBN retention for low-SAPs lubricating oil compositions which have lower starting TBNs.

EP-A-1167497 discloses a lubricating oil composition having a sulphur content of 0.01 to 0.3 wt. % and a phosphorus content of 0.01 to 0.1 wt. %, and giving a sulphated ash content in the range of 0.1 to 1 wt. %, which is said to have good high temperature detergency, and which comprises:
a) a major amount of a mineral base oil having a sulphur content of at most 0.1 wt. %;
b) an ashless dispersant comprising an alkenyl- or alkyl-succinimide or a derivative thereof in an amount of 0.01 to 0.3 wt. % in terms of a nitrogen atom content;
c) a metal-containing detergent containing an organic acid metal salt which is selected from the group consisting of a non-sulphurised alkali metal or alkaline earth metal salt of an alkylsalicylic acid having a TBN of 10 to 350 mg.KOH/g and a non-sulphurised alkali metal or alkaline earth metal salt of an alkylphenol derivative having a Mannich base structure, in an amount of 0.1 to 1 wt. % in terms of a sulphated ash content;
d) a zinc dialkyldithiophosphate in an amount of 0.01 to 0.1 wt. % in terms of a phosphorus content; and
e) an oxidation inhibitor selected from the group consisting of a phenol compound and an amine compound in an amount of 0.01 to 5 wt. %.

The Examples in EP-A-1167497 all use a mixture of 0.7 wt. % aminic antioxidant in combination with 0.7 wt. % phenolic antioxidant.

However, EP-A-1167497 is in no way concerned with the problem of achieving good TBN retention, in particular with regard to the VW T4 test (PV 1449), for compositions having reduced sulphated ash, sulphur and/or phosphorus concentrations therein. In this regard, there is no teaching in EP-A-1167497 to suggest how to achieve good TBN retention in particular with regard to the VW T4 test (PV 1449).

EP-A-1104800 describes a lubricating oil composition for internal combustion engines which comprises
a) a major amount of a base oil of lubricating viscosity,
b) a metal-containing detergent in an amount of 0.1 to 1 wt% in terms of its sulfated ash content,
c) a boron-containing alkenyl- or alkylsuccinimide in an amount of 1.0 to 15 wt% in terms of its active ingredient,
d) a zinc dialkyldithiophosphate in an amount of 0.1 to 0.1 wt% in terms of its phosphorus content,
e) an oxidation inhibitor in an amount of 0.1 to 5 wt% in terms of its active ingredient, and
f) an ashless dithiocarbamate in an amount of 0.1 to 5 wt% in terms of its active ingredient.

US 2003/0148900 A1 discloses a lubricating oil composition for use in natural gas engines which comprises a minor amount of one or more specific hindered phenols and a major amount of at leats one of Group II, III and IV base oils.

US 2003/0148900 A1 indicates that increased amounts of antioxidants may have a detrimental effect on piston deposit control. Accordingly, US 2003/0148900 A1 is directed to a method to increase the oxidation life of lubricating oil base oil without increasing the amount of antioxidant therein.

However, US 2003/0148900 A1 is not concerned with the problem of TBN retention for low-SAPS lubricating oil compositions which have lower starting TBNs.

WO-A-03/083020 describes a method of operating an internal combustion engine that comprises introducing a nitrogen-containing detergent composition into a combustion chamber during the operation of the engine.

Said detergent composition comprises
(A) a reaction product of a hydrocarbyl-substituted acylating agent and an amine;
(B) a hydrocarbyol-substituted amine;
(C) a Mannich reaction product of a hydrocarbyl-substituted hydroxy-containing aromatic compound, an aldehyde, and an amine;
(D) a high molecular weight polyetheramine prepared by reacting one unit of a hydroxy-containing hydrocarbyl compound with two or more units of butylene oxide to form apolyether intermediate, and aminating the polyether intermediate by reacting the polyether intermediate with an amine or with acrylonitrile and hydrogenating the reaction product of the polyether intermediate and acrylnitrile; or
(E) a mixture thereof.

WO 03/099972 discloses a low ash, low phosphorus lubricant composition suitable for use in a stationary gas engine, comprising: (a) an oil of lubricating viscosity; (b) 1.5 to 8 percent by weight of a succinimide dispersant; (c) 0.8 to 4.0 percent by weight of a hindered, ester- substituted phenol antioxidant; and (d) at least one metal-containing sulfonate detergent or metal-containing phenate detergent, in an amount which provides 1.1 to 2.1 percent by weight of said sulfonate or phenate moieties exclusive of the weight of the metal moieties; said lubricant containing up to 0.08 percent by weight phosphorus and up to 1.25 percent sulphated ash.

US-A-5595964 describes a method of lubricating a natural gas-fuelled internal combustion engine, comprising supplying thereto a lubricating oil composition comprising an oil of lubricating viscosity, an antioxidant, an anti-nitration agent and preferably at least about 0.1 wt. % of a borated product of an epoxide, wherein the composition is substantially free of metals and wherein the amount of the antioxidants and the anti-nitration agent are sufficient to reduce the amount of varnish formation in a natural gas-fuelled internal combustion engine.

The total amount of antioxidant used in said lubricating oil composition is said to be at least 1.8 wt. %, preferably at least 2 wt. %.

The lubricating oil composition of US-A-5595964 is said to contain less than 1 % sulphated ash, as determined by ASTM D874.

The phosphorus level of the lubricating oil composition of US-A-5595964 is said to preferably be less than 0.03 % phosphorus, more preferably less than 0.005 % phosphorus.

It is of note that US-A-5595964 is concerned with reducing varnish formation in a natural gas-fuelled internal combustion engine by the presence of an anti-nitration agent in addition to antioxidant in a lubricating oil composition.

US-A-5595964 neither identifies nor addresses the problem of poor TBN retention in lubricating oil compositions having reduced sulphated ash, sulphur and/or phosphorus concentrations therein, and in particular in low-SAPS lubricating oil compositions which have lower starting TBNs. There is no disclosure in US-A-5595964 to suggest how to achieve good TBN retention in such lubricating oil compositions, particularly in order to pass the VW T4 test (PV 1449).

It is therefore desirable to develop lubricating oil compositions having reduced sulphated ash, sulphur and/or phosphorus concentrations therein which have good TBN retention, and in particular low SAPS lubricating oil compositions which have lower starting TBNs and which have good TBN retention.

It is particularly desirable to develop such lubricating oil compositions which have good TBN retention with regard to the VW T4 test (PV 1449), more particularly to develop such lubricating oil compositions having an end of test (VW T4 Test (PV 1449)) TBN value of at least 5.0 mg.KOH/g, as measured by ISO 3771.

There has now been surprisingly found in the present invention, a lubricating oil composition having a low sulphated ash content which is suitable for lubricating internal combustion engines and which exhibits advantageous TBN retention properties.

Accordingly, the present invention provides a use of a lubricating oil composition to maintain a TBN level of at least 5.0 mg.KOH/g, as measured by ISO 3771, in an internal combustion engine in the VW T4 Test (PV 1449), wherein said lubricating oil composition has a sulphated ash content of not greater than 0.9 wt. % and a phosphorus content in the range of from 0.04 to 0.1 wt. %, and said lubricating oil composition comprises base oil,
(A) one or more detergents selected from phenate detergents, salicylate detergents and sulphonate detergents, wherein said one or more detergents each, independently, have a TBN (total base number) value in the range of from 30 to 350 mg.KOH/g, as measured by ISO 3771; and
(B) at least 3.5 wt. % of one or more antioxidants, based on the total weight of the lubricating oil composition,wherein the one or more antioxidants in said lubricating oil composition comprise aminic antioxidants.

In a preferred embodiment, said one or more antioxidants are present in an amount of at least 3.7 wt. %, more preferably in an amount of at least 3.9 wt. %, and most preferably in an amount of at least 4.0 wt. %, based on the total weight of the lubricating oil composition.

The lubricating oil composition used in the present invention comprises one or more aminic antioxidants.

Examples of aminic antioxidants which may be conveniently used include alkylated diphenylamines, phenyl-α-naphthylamines, phenyl-β-naphthylamines and alkylated α-naphthylamines.

Preferred aminic antioxidants include dialkyldiphenylamines such as p,p'-dioctyl-diphenylamine, p,p'-di-α-methylbenzyl-diphenylamine and N-p-butylphenyl-N-p'-octylphenylamine, monoalkyldiphenylamines such as mono-t-butyldiphenylamine and mono-octyldiphenylamine, bis(dialkylphenyl)amines such as di-(2,4-diethylphenyl)amine and di(2-ethyl-4-nonylphenyl)amine, alkylphenyl-1-naphthylamines such as octylphenyl-1-naphthylamine and n-t-dodecylphenyl-1-naphthylamine, 1-naphthylamine, arylnaphthylamines such as phenyl-1-naphthylamine, phenyl-2-naphthylamine, N-hexylphenyl-2-naphthylamine and N-octylphenyl-2-naphthylamine, phenylenediamines such as N,N'-diisopropyl-p-phenylenediamine and N,N'-diphenyl-p-phenylenediamine, and phenothiazines such as phenothiazine and 3,7-dioctylphenothiazine.

Preferred aminic antioxidants include those available under the following trade designations: "Sonoflex OD-3" (ex. Seiko Kagaku Co.), "Irganox L-57" (ex. Ciba Specialty Chemicals Co.) and phenothiazine (ex. Hodogaya Kagaku Co.).

The lubricating oil composition used in the present invention may comprise one or more phenolic antioxidants.

Examples of phenolic antioxidants which may be conveniently used include C7-C9 branched alkyl esters of 3,5-bis(1,1-dimethyl-ethyl)-4-hydroxy-benzenepropanoic acid, 2-t-butylphenol, 2-t-butyl-4-methylphenol, 2-t-butyl-5-methylphenol, 2,4-di-t-butylphenol, 2,4-dimethyl-6-t-butylphenol, 2-t-butyl-4-methoxyphenol, 3-t-butyl-4-methoxyphenol, 2,5-di-t-butylhydroquinone, 2,6-di-t-butyl-4-alkylphenols such as 2,6-di-t-butylphenol, 2,6-di-t-butyl-4-methylphenol and 2,6-di-t-butyl-4-ethylphenol, 2,6-di-t-butyl-4-alkoxyphenols such as 2,6-di-t-butyl-4-methoxyphenol and 2,6-di-t-butyl-4-ethoxyphenol, 3,5-di-t-butyl-4-hydroxybenzylmercaptooctylacetate, alkyl-3(3,5-di-t-butyl-4-hydroxyphenyl)propionates such as n-octadecyl-3-(3,5-di-t-butyl-4-hydroxyphenyl)propionate, n-butyl-3-(3,5-di-t-butyl-4-hydroxyphenyl)propionate and 2'-ethylhexyl-3-(3,5-di-t-butyl-4-hydroxyphenyl)propionate, 2,6-d-t-butyl-α-dimethylamino-p-cresol, 2,2'-methylene-bis(4-alkyl-6-t-butylphenol) such as 2,2'-methylenebis(4-methyl-6-t-butylphenol, and 2,2-methylenebis(4-ethyl-6-t-butylphenol), bisphenols such as 4,4'-butylidenebis(3-methyl-6-t-butylphenol, 4,4'-methylenebis(26-di-t-butylphenol), 4,4'-bis(2,6-di-t-butylphenol), 2,2-(di-p-hydroxyphenyl)propane, 2,2-bis(3,5-di-t-butyl-4-hydroxyphenyl)propane, 4,4'-cyclohexylidenebis(2,6-t-butylphenol), hexamethyleneglycol-bis[3-(3,5-di-t-butyl-4-hydroxyphenyl)propionate], triethyleneglycolbis[3-(3-t-butyl-4-hydroxy-5-methylphenyl)propionate], 2,2'-thio-[diethyl-3-(3,5-di-t-butyl-4-hydroxyphenyl)propionate], 3,9-bis{1,1-dimethyl-2-[3-(3-t-butyl-4-hydroxy-5-methylphenyl)propionyloxy]ethyl}2,4,8,10-tetraoxaspiro[5,5]undecane, 4,4'-thiobis(3-methyl-6-t-butylphenol) and 2,2'-thiobis(4,6-di-t-butylresorcinol), polyphenols such as tetrakis[methylene-3-(3,5-di-t-butyl-4-hydroxyphenyl)propionate]methane, 1,1,3-tris(2-methyl-4-hydroxy-5-t-butylphenyl)butane, 1,3,5-trimethyl-2,4,6-tris(3,5-di-t-butyl-4-hydroxybenzyl)benzene, bis-[3,3'-bis(4'-hydroxy-3'-t-butylphenyl)butyric acid]glycol ester, 2-(3',5'-di-t-butyl-4-hydroxyphenyl)methyl-4-(2",4"-di-t-butyl-3"-hydroxyphenyl)methyl-6-t-butylphenol and 2,6-bis(2'-hydroxy-3'-t-butyl-5'-methylbenzyl)-4-methylphenol, and p-t-butylphenol - formaldehyde condensates and p-t-butylphenol - acetaldehyde condensates.

Preferred phenolic antioxidants include those available under the following trade designations: "Irganox L-135" (ex. Ciba Specialty Chemicals Co.), "Anteeji DBH" (ex. Kawaguchi Kagaku Co.,), "Yoshinox SS" (ex. Yoshitomi Seiyaku Co.), "Antage W-400" (ex. Kawaguchi Kagaku Co.), "Antage W-500" (ex. Kawaguchi Kagaku Co.), "Antage W-300" (ex. Kawaguchi Kagaku Co.), "Ionox 220AH" (ex. Shell Japan Co.), bisphenol A, produced by the Shell Japan Co., "Irganox L109" (ex. Ciba Speciality Chemicals Co.), "Tominox 917" (ex. Yoshitomi Seiyaku Co.), "Irganox L115" (ex. Ciba Speciality Chemicals Co.), "Sumilizer GA80" (ex. Sumitomo Kagaku), "Antage RC" (ex. Kawaguchi Kagaku Co.), "Irganox L101" (ex. Ciba Speciality Chemicals Co.), "Yoshinox 930" (ex. Yoshitomi Seiyaku Co.), "Ionox 330" (ex. Shell Japan Co.).

The lubricating oil composition herein may comprise mixtures of one or more phenolic antioxidants with one or more aminic antioxidants.

Detergents that may be used in the lubricating oil herein include one or more detergents selected from salicylate detergents, phenate detergents and sulphonate detergents.

Alkali metal and alkaline earth metal salicylate, phenate and sulphonate detergents are preferred in the lubricating oil compositions herein. Calcium and magnesium salicylates, phenates and sulphonates are particularly preferred detergents therein.

In one embodiment, the lubricating oil composition herein may comprise (i) one or more salicylate detergents; and/or (ii) a mixture of one or more phenate detergents and one or more sulphonate detergents.

However, as metal organic and inorganic base salts which are used as detergents can contribute to the sulphated ash content of a lubricating composition, in a preferred embodiment of the present invention, the amounts of such detergent additives are minimised.

In order to maintain a low sulphur level, salicylate detergents are particularly preferred.

Thus, in a preferred embodiment, the lubricating oil composition herein may comprise one or more salicylate detergents.

In order to maintain the total sulphated ash content of the lubricating oil composition herein at a level of not greater than 0.9 wt. %, preferably at a level of not greater than 0.8 wt. %, more preferably at a level of not greater than 0.75 wt. % and most preferably at a level of not greater than 0.7 wt. %, based on the total weight of the lubricating oil composition, said one or more detergents (A) are preferably used in amounts in the range of 0.05 to 12.5 wt. %, more preferably from 1.0 to 9.0 wt. % and most preferably in the range of from 2.0 to 5.0 wt. %, based on the total weight of the lubricating oil composition.

Furthermore, it is preferred that said one or more detergents (A), each, independently, have a TBN (total base number) value in the range of from 30 to 350 mg.KOH/g, more preferably in the range of from 50 to 300 mg.KOH/g, as measured by ISO 3771.

That is to say, when there is more than one detergent selected from phenate detergents, salicylate detergents and sulphonate detergents present in the lubricating oil composition herein, then each of such detergents will have a TBN (total base number) value in the range of from 30 to 350 mg.KOH/g, more preferably in the range of from 50 to 300 mg.KOH/g, as measured by ISO 3771.

The amount of base oil incorporated in the lubricating oil composition herein is preferably present in an amount in the range of from 60 to 92 wt. %, more preferably in an amount in the range of from 75 to 90 wt. % and most preferably in an amount in the range of from 75 to 88 wt. %, with respect to the total weight of the lubricating oil composition.

There are no particular limitations regarding the base oil used in the present invention, and various conventional known mineral oils and synthetic lubricating oils may be conveniently used.

Mineral oils include liquid petroleum oils and solvent-treated or acid-treated mineral lubricating oil of the paraffinic, naphthenic, or mixed paraffinic/naphthenic type which may be further refined by hydrofinishing processes and/or dewaxing.

Naphthenic base oils have low viscosity index (VI) (generally 40-80) and a low pour point. Such base oils are produced from feedstocks rich in naphthenes and low in wax content and are used mainly for lubricants in which colour and colour stability are important, and VI and oxidation stability are of secondary importance.

Paraffinic base oils have higher VI (generally >95) and a high pour point. Said base oils are produced from feedstocks rich in paraffins, and are used for lubricants in which VI and oxidation stability are important.

Fischer-Tropsch derived base oils may be conveniently used as the base oil in the lubricating oil composition herein, for example, the Fischer-Tropsch derived base oils disclosed in EP-A-776959, EP-A-668342, WO-A-97/21788, WO-00/15736, WO-00/14188, WO-00/14187, WO-00/14183, WO-00/14179, WO-00/08115, WO-99/41332, EP-1029029, WO-01/18156 and WO-01/57166.

Synthetic processes enable molecules to be built from simpler substances or to have their structures modified to give the precise properties required.

Synthetic lubricating oils include hydrocarbon oils such as olefin oligomers (PAOs), dibasic acids esters, polyol esters, and dewaxed waxy raffinate. Synthetic hydrocarbon base oils sold by the Royal Dutch/Shell Group of Companies under the designation "XHVI" (trade mark) may be conveniently used.

Preferably, the base fluid constituted from mineral oils and/or synthetic base oils which contain more than 80% wt of saturates, preferably more than 90 % wt., as measured according to ASTM D2007.

It is further preferred that the base oil contains less than 1.0 wt. %, preferably less than 0.1 wt. % of sulphur, calculated as elemental sulphur and measured according to ASTM D2622, ASTM D4294, ASTM D4927 or ASTM B3120.

Preferably, the viscosity index of base fluid is more than 80, more preferably more than 120, as measured according to ASTM D2270.

Preferably, the lubricating oil has a kinematic viscosity in the range of from 2 to 80 mm²/s at 100 °C, more preferably of from 3 to 70 mm²/s, most preferably of from 4 to 50 mm²/s.

In a preferred embodiment, the lubricating oil composition may comprise a single zinc dithiophosphate or a combination of two or more zinc dithiophosphates as anti-wear additives, the or each zinc dithiophosphate being selected from zinc dialkyl-, diaryl- or alkylaryl- dithiophosphates.

Zinc dithiophosphate is a well known additive in the art and may be conveniently represented by general formula II; wherein R² to R⁵ may be the same or different and are each a primary alkyl group-containing from 1 to 20 carbon atoms preferably from 3 to 12 carbon atoms, a secondary alkyl group containing from 3 to 20 carbon atoms, preferably from 3 to 12 carbon atoms, an aryl group or an aryl group substituted with an alkyl group, said alkyl substituent containing from 1 to 20 carbon atoms preferably 3 to 18 carbon atoms.

Zinc dithiophosphate compounds in which R² to R⁵ are all different from each other can be used alone or in admixture with zinc dithiophosphate compound in which R² to R⁵ are all the same.

Preferably, the or each zinc dithiophosphate used in the present invention is a zinc dialkyl dithiophosphate.

Examples of suitable zinc dithiophosphates which are commercially available include those available ex. Lubrizol Corporation under the trade designations "Lz 1097" and "Lz 1395", those available ex. Chevron Oronite under the trade designations "OLOA 267" and "OLOA 269R", and that available ex. Ethyl under the trade designation "HITEC 7197"; zinc dithiophosphates such as those available ex. Lubrizol Corporation under the trade designations "Lz 677A", "Lz 1095" and "Lz 1371", that available ex. Chevron Oronite under the trade designation "OLOA 262" and that available ex. Ethyl under the trade designation "HITEC 7169"; and zinc dithiophosphates such as those available ex. Lubrizol Corporation under the trade designations "Lz 1370" and "Lz 1373" and that available ex. Chevron Oronite under the trade designation "OLOA 260".

The lubricating oil composition herein may generally comprise in the range of from 0.4 to 1.0 wt. % of zinc dithiophosphate, (if primary or secondary alkyl type), preferably in the range of from 0.4 to 0.9 wt. % and most preferably in the range of from 0.45 to 0.8 wt. %, based on total weight of the lubricating oil composition.

The total amount of phosphorus in the lubricating oil composition herein is therefore generally in the range of from 0.04 to 0.1 wt. %, more preferably in the range of from 0.04 to 0.09 wt. % and most preferably in the range of from 0.045 to 0.08 wt. %, based on total weight of the lubricating oil composition.

At phosphorus levels of 0.04 wt. % and below, there may be insufficient anti-wear performance. At phosphorus levels of 0.1 wt. % and above, the phosphorus may have a detrimental effect on vehicle exhaust after-treatment devices.

The lubricating oil composition herein preferably has a sulphated ash content of not greater than 0.8 wt. %, more preferably not greater than 0.75 wt. % and most preferably not greater than 0.7 wt. %, based on the total weight of the lubricating oil composition.

The lubricating oil composition herein preferably has a sulphur content of not greater than 1.2 wt. %, more preferably not greater than 0.8 wt. % and most preferably not greater than 0.2 wt. %, based on the total weight of the lubricating oil composition.

Preferred compositions herein have one or more of the following features:
(i) greater than 0.04 wt. % of phosphorus;
(ii) greater than 0.045 wt. % of phosphorus;
(iii) at least 0.04 wt. % of phosphorus;
(iv) less than 0.09 wt. % of phosphorus;
(v) not greater than 0.10 wt. % of phosphorus;
(vi) at most 0.08 wt. % of phosphorus;
(vii) not greater than 0.9 wt. % of sulphated ash;
(viii) not greater than 0.8 wt. % of sulphated ash;
(ix) not greater than 0.7 wt. % of sulphated ash;
(x) not greater than 1.2 wt. % of sulphur;
(xi) not greater than 0.8 wt. % of sulphur; and
(xii) not greater than 0.2 wt. % of sulphur, based on the total weight of the lubricating oil composition.

Particularly preferred compositions herein are:-
(A): those having features (i) and (iv); those having features (i) and (v); those having features (i) and (vi); those having features (ii) and (iv); those having features (ii) and (v); those having features (ii) and (vi); those having features (iii) and (iv); those having features (iii) and (v); and those having features (iii) and (vi);
(B): those having features (i), (iv) and (vii); those having features (i), (iv) and (viii); those having features (i), (iv) and (ix); those having features (i), (v) and (vii); those having features (i), (v) and (viii); those having features (i), (v) and (ix); those having features (i), (vi) and (vii); those having features (i), (vi) and (viii); those having features (i), (vi) and (ix); those having features (ii), (iv) and (vii); those having features (ii), (iv) and (viii); those having features (ii), (iv) and (ix); those having features (ii), (v) and (vii); those having features (ii), (v) and (viii); those having features (ii), (v) and (ix); those having features (ii), (vi) and (vii); those having features (ii), (vi) and (viii); those having features (ii), (vi) and (ix); those having features (iii), (iv) and (vii); those having features (iii), (iv) and (viii); those having features (iii), (iv) and (ix); those having features (iii), (v) and (vii); those having features (iii), (v) and (viii); those having features (iii), (v) and (ix); those having features (iii), (vi) and (vii); those having features (iii), (vi) and (viii); and those having features (iii), (vi) and (ix);
(C): those having features (i), (iv) and (x); those having features (i), (iv) and (xi); those having features (i), (iv) and (xii); those having features (i), (v) and (x); those having features (i), (v) and (xi); those having features (i), (v) and (xii); those having features (i), (vi) and (x); those having features (i), (vi) and (xi); those having features (i), (vi) and (xii); those having features (ii), (iv) and (x); those having features (ii), (iv) and (xi); those having features (ii), (iv) and (xii); those having features (ii), (v) and (x); those having features (ii), (v) and (xi); those having features (ii), (v) and (xii); those having features (ii), (vi) and (x); those having features (ii), (vi) and (xi); those having features (ii), (vi) and (xii); those having features (iii), (iv) and (x); those having features (iii), (iv) and (xi); those having features (iii), (iv) and (xii); those having features (iii), (v) and (x); those having features (iii), (v) and (xi); those having features (iii), (v) and (xii); those having features (iii), (vi) and (x); those having features (iii), (vi) and (xi); and those having features (iii), (vi) and (xii); and
(D): those having features (i), (iv), (vii) and (x); those having features (i), (iv), (viii) and (x); those having features (i), (iv), (ix) and (x); those having features (i), (v), (vii) and (x); those having features (i), (v), (viii) and (x); those having features (i), (v), (ix) and (x); those having features (i), (vi), (vii) and (x); those having features (i), (vi), (viii) and (x); those having features (i), (vi), (ix) and (x); those having features (ii), (iv), (vii) and (x); those having features (ii), (iv), (viii) and (x): those having features (ii), (iv), (ix) and (x); those having features (ii), (v), (vii) and (x); those having features (ii), (v), (viii) and (x); those having features (ii), (v), (ix) and (x); those having features (ii), (vi), (vii) and (x); those having features (ii), (vi), (viii) and (x); those having features (ii), (vi), (ix) and (x); those having features (iii), (iv), (vii) and (x); those having features (iii), (iv), (viii) and (x); those having features (iii), (iv), (ix) and (x); those having features (iii), (v), (vii) and (x); those having features (iii), (v), (viii) and (x); those having features (iii), (v), (ix) and (x); those having features (iii), (vi), (vii) and (x); those having features (iii), (vi), (viii) and (x); those having features (iii), (vi), (ix) and (x); those having features (i), (iv), (vii) and (xi); those having features (i), (iv), (viii) and (xi); those having features (i), (iv), (ix) and (xi); those having features (i), (v); (vii) and (xi); those having features (i), (v), (viii) and (xi); those having features (i), (v), (ix) and (xi); those having features (i), (vi), (vii) and (xi); those having features (i), (vi), (viii) and (xi); those having features (i), (vi), (ix) and (xi); those having features (ii), (iv), (vii) and (xi); those having features (ii), (iv), (viii) and (xi); those having features (ii), (iv), (ix) and (xi); those having features (ii), (v), (vii) and (xi); those having features (ii), (v), (viii) and (xi); those having features (ii), (v), (ix) and (xi); those having features (ii), (vi), (vii) and (xi); those having features (ii), (vi), (viii) and (xi); those having features (ii), (vi), (ix) and (xi); those having features (iii), (iv), (vii) and (xi); those having features (iii), (iv), (viii) and (xi); those having features (iii), (iv), (ix) and (xi); those having features (iii), (v), (vii) and (xi); those having features (iii), (v), (viii) and (xi); those having features (iii), (v), (ix) and (xi); those having features (iii), (vi), (vii) and (xi); those having features (iii), (vi), (viii) and (xi); those having features (iii), (vi), (ix) and (xi); those having features (i), (iv), (vii) and (xii); those having features (i), (iv), (viii) and (xii); those having features (i), (iv), (ix) and (xii); those having features (i), (v), (vii) and (xii); those having features (i), (v), (viii) and (xii); those having features (i), (v), (ix) and (xii); those having features (i), (vi), (vii) and (xii); those having features (i), (vi), (viii) and (xii); those having features (i), (vi), (ix) and (xii); those having features (ii), (iv), (vii) and (xii); those having features (ii), (iv), (viii) and (xii); those having features (ii), (iv), (ix) and (xii); those having features (ii), (v), (vii) and (xii); those having features (ii), (v), (viii) and (xii); those having features (ii), (v), (ix) and (xii); those having features (ii), (vi), (vii) and (xii); those having features (ii), (vi), (viii) and (xii); those having features (ii), (vi), (ix) and (xii); those having features (iii), (iv), (vii) and (xii); those having features (iii), (iv), (viii) and (xii); those having features (iii), (iv), (ix) and (xii); those having features (iii), (v), (vii) and (xii); those having features (iii), (v), (viii) and (xii); those having features (iii), (v), (ix) and (xii); those having features (iii), (vi), (vii) and (xii); those having features (iii), (vi), (viii) and (xii); and those having features (iii), (vi), (ix) and (xii).

The lubricating oil composition herein may further comprise additional additives such as supplementary anti-wear additives, supplementary detergents, dispersants, friction modifiers, viscosity index improvers, pour point depressants, corrosion inhibitors, defoaming agents and seal fix or seal compatibility agents.

Supplementary anti-wear additives that may be conveniently used include molybdenum-containing compounds and boron-containing compounds.

Examples of such molybdenum-containing compounds may conveniently include molybdenum dithiocarbamates, trinuclear molybdenum compounds, for example as described in WO-A-98/26030, sulphides of molybdenum and molybdenum dithiophosphate.

Said molybdenum-containing anti-wear additives may be conveniently added to the lubricating oil composition herein in an amount in the range of from 0.1 to 3.0 wt. %, based on the total weight of lubricating oil composition.

Boron-containing compounds that may be conveniently used include borate esters, borated fatty amines, borated epoxides, alkali metal (or mixed alkali metal or alkaline earth metal) borates and borated overbased metal salts.

Said boron-containing anti-wear additives may be conveniently added to the lubricating oil composition herein in an amount in the range of from 0.1 to 3.0 wt. %, based on the total weight of lubricating oil composition.

The TBN value of fresh unused samples of the lubricating oil composition herein is preferably in the range of from 5.0 to 12.0 mg.KOH/g, more preferably in the range of from 6.0 to 11.0 mg.KOH/g, even more preferably in the range of from 6.0 to 10.0 mg.KOH/g and most preferably in the range of 6.0 to 9.0 mg.KOH/g, as measured by ISO 3771.

The lubricating oil compositions herein may additionally contain an ash-free dispersant which is preferably admixed in an amount in the range of from 5 to 15 wt. %, based on the total weight of the lubricating oil composition.

Examples of dispersants which may be used include the polyalkenyl succinimides and polyalkenyl succininic acid esters disclosed in Japanese Patent Nos. 1367796, 1667140, 1302811 and 1743435. Preferred dispersants include borated succinimides.

Preferred friction modifiers that may be conveniently used include fatty acid amides, more preferably unsaturated fatty acid amides.

The total amount of friction modifiers added to the lubricating oil composition herein is conveniently in the range of from 0.05 to 1.2 wt. %, based on the total weight of the lubricating oil composition.

Examples of viscosity index improvers which may conveniently be used in the lubricating oil composition herein include the styrene-butadiene copolymers, styreneisoprene stellate copolymers and the polymethacrylate-based and ethylene-propylene copolymers and the like disclosed in Japanese Patent Nos. 954077, 1031507, 1468752, 1764494 and 1751082. Such viscosity index improvers may be conveniently employed in an amount in the range of from 1 to 20 wt. %, based on the total weight of the lubricating oil composition. Similarly, dispersing-type viscosity index improvers comprising copolymerized polar monomer containing nitrogen atoms and oxygen atoms in the molecule may also be used therein.

Polymethacrylates such as those as disclosed in Japanese Patent Nos. 1195542 and 1264056 may be conveniently employed in the lubricating oil compositions herein as effective pour point depressants.

Furthermore, compounds such as alkenyl succinic acid or ester moieties thereof, benzotriazole-based compounds and thiodiazole-based compounds may be conveniently used in the lubricating oil composition herein as corrosion inhibitors.

Compounds such as polysiloxanes, dimethyl polycyclohexane and polyacrylates may be conveniently used in the lubricating oil composition herein as defoaming agents.

Compounds which may be conveniently used in the lubricating oil composition herein as seal fix or seal compatibility agents include, for example, commercially available aromatic esters.

The lubricating oil compositions herein may be conveniently prepared by admixing the one or more detergents (A), the one or more antioxidants (B) selected from phenolic and/or aminic antioxidants, and, optionally, one or more further additives that are usually present in lubricating oils, for example as herein before described, with a mineral and/or synthetic base oil.

Lubricating oil compositions herein display advantageous TBN retention, in particular with regard to the VW T4 test (PV 1449).

In a preferred embodiment of the present invention, the end of test (VW T4 Test (PV 1449)) TBN value is at least 5.0 mg.KOH/g, as measured by ISO 3771.

In a preferred embodiment of the present invention, the TBN value of a fresh unused sample of the lubricating oil composition herein is in the range of from 5.0 to 12.0 mg.KOH/g and the end of test (VW T4 Test (PV 1449)) TBN value of the same lubricating oil composition is at least 5.0 mg.KOH/g, as measured by ISO 3771.

In another preferred embodiment of the present invention, the TBN value of a fresh unused sample of the lubricating oil composition herein is in the range of from 6.0 to 11.0 mg.KOH/g and the end of test (VW T4 Test (PV 1449)) TBN value of the same lubricating oil composition is at least 6.0 mg.KOH/g, as measured by ISO 3771.

In yet another preferred embodiment of the present invention, the TBN value of a fresh unused sample of the lubricating oil composition herein is in the range of from 6.0 to 10.0 mg.KOH/g and the end of test (VW T4 Test (PV 1449)) TBN value of the same lubricating oil composition is at least 6.0 mg.KOH/g, as measured by ISO 3771.

In the present invention, it is preferred that the change in TBN between the TBN of a fresh unused sample of the lubricating oil composition herein and the end of test (VW T4 Test (PV 1449)) TBN value of the same lubricating oil composition (i.e. wherein ΔTBN is the TBN of fresh oil - End of test TBN) is less than 2.5 mg.KOH/g, more preferably less than 2.0 mg KOH/g and most preferably less than 1.8 mg.KOH/g.

In a preferred embodiment of the present invention, the end of test (VW T4 Test (PV 1449)) Vk40 value (i.e. kinematic viscosity at 40 °C) is less than 200 mm²/s (cSt).

Accordingly, there is provided the use of a lubricating oil composition as hereinbefore described to maintain a TBN level of at least 5.0 mg.KOH/g, as measured by ISO 3771, in an internal combustion engine, in particular with regard to the VW T4 test (PV 1449).

The present invention is described below with reference to the following Examples, which are not intended to limit the scope of the invention in any way.

### EXAMPLES

### Formulations

Table 1 indicates the formulations that were tested.

The formulations in Table 1 comprised conventional detergents, antifoam, dispersants, pour point depressants, viscosity index modifiers and zinc dithiophosphate additives, which were present as additive packages in diluent oil.

The phenolic antioxidant used was that available under the trade designation "Irganox L-135" ex. Ciba Specialty Chemicals Co. (C7-C9 branched alkyl esters of 3,5-bis(1,1-dimethyl-ethyl)-4-hydroxy-benzenepropanoic acid).

The aminic antioxidant used was that available under the trade designation "Irganox L-57" ex. Ciba Speciality Chemicals Co.

The base oils used in said formulations were mixtures of Group III base oils available from "The Royal Dutch/Shell Group of Companies" under the trade designations "XHVI-5.2" and "XHVI-8.2".

All formulations described in Table 1 were SAE 5W30 viscosity grade oils.

Table 2 indicates the physical characteristics of the formulations that were tested.

**TABLE 1**

| **Additive (wt. %)** | **Ex. 1*** | **Ex. 2*** | **Ex. 3*** | **Ex. 4*** | **Ex. 5*** | **Ex. 6** | **Comp. Ex. 1*** |
|---|---|---|---|---|---|---|---|
| Anti-foam | 30ppm | 30ppm | 30ppm | 30ppm | 30ppm | 30 ppm | 30ppm |
| Additive package A¹ | 14.0 | - | - | - | - | 14.0 | 14.0 |
| Additive Package B² | - | 10.9 | - | - | - | - | - |
| Additive Package C³ | - | - | 10.1 | - | - | - | - |
| Additive Package D⁴ | - | - | - | 10.7 | - | - | - |
| Additive Package E⁵ | - | - | - | - | 11.5 | - | - |
| Phenolic Antioxidant | 4.0 | 4.0 | 4.0 | 4.0 | 4.0 | - | - |
| Aminic Antioxidant | - | - | - | - | - | 4.0 | - |
| Viscosity modifier⁶ | 9.60 | 12.0 | 12.0 | 12.0 | 12.0 | 9.60 | 9.60 |
| Pour point depressant | 0.3 | - | - | - | - | 0.3 | 0.3 |
| Base oil⁷ | 72.10 | 73.10 | 73.90 | 73.80 | 72.50 | 72.10 | 76.10 |
| **TOTAL** | 100 | 100 | 100 | 100 | 100 | 100 | 100 |

| | | | | | | | |
|---|---|---|---|---|---|---|---|
| *Comparative Examples ¹ Commercial additive package available ex. Lubrizol under the trade designation "LZ OS183698", containing sulphonate and phenate detergents each having TBNs in the range of from 30 to 350 mg.KOH/g, dispersant, zinc dithiophosphate and diluent oil. ² Conventional additive package containing calcium salicylate detergents having TBNs of 165 mg.KOH/g and 280 mg.KOH/g, dispersant, zinc dithiophosphate and diluent oil. ³ Conventional additive package containing magnesium salicylate detergent having a TBN of 345 mg.KOH/g, dispersant, zinc dithiophosphate and diluent oil. ⁴ Conventional additive package containing magnesium salicylate detergent having a TBN of 345 mg.KOH/g, dispersant, zinc dithiophosphate and diluent oil. ⁵ Conventional additive package containing calcium salicylate detergents having TBNs of 64 mg.KOH/g and 165 mg.KOH/g, dispersant, zinc dithiophosphate and diluent oil. ⁶ Mixture of two different viscosity index modifiers. ⁷ Group III base oil mixtures of XHVI-5.2 and XHVI-8.2 | | | | | | | |

**TABLE 2**

| **Analytical Measurements** | Total Sulphated ash | Total Sulphur | Total Phosphorus | Ca | Mg |
|---|---|---|---|---|---|
| | (wt. %) (ASTM D874) | (wt. %) (ASTM D2622) | (wt. %) (ICP-OES method) | (wt. %) (ICP-OES method) | (wt.%) (ICP-OES method) |
| **Ex. 1*** | 0.77 | 0.188 | 0.068 | 0.163 | 0 |
| **Ex. 2*** | 0.85 | 0.186 | 0.047 | 0.207 | 0 |
| **Ex. 3*** | 0.64 | 0.125 | 0.050 | 0 | 0.118 |
| **Ex. 4*** | 0.85 | 0.131 | 0.049 | 0 | 0.163 |
| **Ex. 5*** | 0.63 | 0.135 | 0.050 | 0.150 | 0 |
| **Ex. 6** | 0.82 | 0.183 | 0.072 | 0.166 | 0 |
| **Comp. Ex. 1*** | 0.76 | 0.131 | 0.074 | 0.167 | 0 |

| | | | | | |
|---|---|---|---|---|---|
| *Comparative Examples | | | | | |

VW T4 test (PV 1449)

The experimental methodology used for the Examples above was in accordance with the publicly available test specification for the VW T4 test (PV 1449) and as described in the standard test methods referred to in said test specification.

### Results and Discussion

The formulations described in Tables 1 and 2 were tested using the afore-mentioned test and the results obtained thereon are included in Table 3.

**TABLE 3**

| **Test Results** | **Ex. 1¹** | **Ex. 2¹** | **Ex. 3¹** | **Ex. 4¹** | **Ex. 5¹** | **Ex. 6** | **Comp. Ex. 1¹** |
|---|---|---|---|---|---|---|---|
| Vk40* increase (%) | 125.5 | 73.9 | 69 | 74.4 | 77.2 | 114.1 | 98 |
| Vk40 at end of test** (mm²/s) | 144.6 | 121 | 117.8 | 121.2 | 122.8 | 141.7 | 135.4 |
| (1) TBN of fresh oil (mg.KOH/g) (ISO 3771) | 7.8 | 8.0 | 7.6 | 9.4 | 5.9 | 5.28 | 6.9 |
| (2) End of test TBN*** (mg.KOH/g) (ISO 3771) | 6.1 | 7.3 | 6.2 | 8.1 | 5.1 | 5.12 | 3.6 |
| Δ TBN**** (mg.KOH/g) | 1.7 | 0.7 | 1.4 | 1.3 | 0.8 | 0.16 | 3.3 |
| % change in TBN | -21.7 | -8.8 | -18.4 | -13.8 | -13.6 | -3.0 | -47.3 |

| | | | | | | | |
|---|---|---|---|---|---|---|---|
| * Kinematic viscosity at 40 °C. ** End of Test Limit (VW T4 test (PV 1449)) is <200 (mm²/s). *** End of Test Limit (VW T4 test (PV 1449)) is 5.0 mg.KOH/g. **** TBN of fresh oil - End of test TBN. ¹ Comparative Examples | | | | | | | |

It is evident from the above results that the formulation of Example 1 which comprises a phenolic antioxidant, displays increased TBN retention according to the VW T4 test (PV 1449), as compared with the formulation of Comparative Example 1 which fails to meet the required minimum end of test TBN result of 5.0 mg.KOH/g.

Furthermore, the formulations or Examples 2 to 5 which also contain large amounts of phenolic antioxidant, also surprisingly pass the VW T4 test (PV 1449) end of test TBN limit of 5.0 mg.KOH/g.

It is further evident that the formulation of Example 6 which comprises an aminic antioxidants, also displays increased TBN retention according to the VW T4 test (PV 1449), as compared with the formulation of Comparative Example 1.

## Claims

1. Use of a lubricating oil composition to maintain a TBN level of at least 5.0 mg.KOH/g, as measured by ISO 3771, in an internal combustion engine in the VW T4 Test (PV 1449), wherein said lubricating oil composition has a sulphated ash content of not greater than 0.9 wt. % and a phosphorus content in the range of from 0.04 to 0.1 wt. %, and said lubricating oil composition comprises base oil,
(A) one or more detergents selected from phenate detergents, salicylate detergents and sulphonate detergents, wherein said one or more detergents each, independently, have a TBN (total base number) value in the range of from 30 to 350 mg.KOH/g, as measured by ISO 3771; and
(B) at least 3.5 wt. % of one or more antioxidants, based on the total weight of the lubricating oil composition, wherein the one or more antioxidants in said lubricating oil composition comprise aminic antioxidants.

2. Use according to Claim 1, wherein said one or more antioxidants are present in said lubricating oil composition an amount of at least 3.7 wt. %, based on the total weight of the lubricating oil composition.

3. Use according to Claim 1 or 2, wherein said one or more aminic antioxidants are selected from alkylated diphenylamines, phenyl-α-naphthylamines, phenyl-β-naphthylamines and alkylated α-naphthylamines.

4. Use according to any one of Claims 1 to 3, wherein the lubricating oil composition has a sulphur content of not greater than 1.2 wt. %, based on the total weight of the lubricating oil composition.

5. Use according to any one of Claims 1 to 4, wherein the lubricating oil composition has a phosphorus content in the range of from 0.04 to 0.09 wt. %, based on the total weight of the lubricating oil composition.

6. Use according to any one of Claims 1 to 5, wherein the TBN value of a fresh unused sample of the lubricating oil composition is in the range of from 5.0 to 12.0 mg.KOH/g, as measured by ISO 3771.

7. Use according to any one of Claims 1 to 6, wherein the change in TBN value of a fresh unused sample of the lubricating oil composition, as measured by ISO 3771, and the end of test (VW T4 Test (PV 1449)) TBN value of the same lubricating oil composition, as measured by ISO 3771, is less than 2.5 mg.KOH/g.

## Patentansprüche

1. Verwendung einer Schmierölzusammensetzung, um einen TBN-Wert von zumindest 5,0 mg.KOH/g, gemessen nach ISO 3771, in einem Verbrennungsmotor in dem VW-T4-Test (PV 1449) konstant zu halten, wobei die Schmierölzusammensetzung einen Sulfataschegehalt von nicht größer als 0,9 Gew.-% und einen Phosphorgehalt im Bereich von 0,04 bis 0,1 Gew.-% aufweist und wobei die Schmierölzusammensetzung ein Basisöl umfasst,
(A) ein oder mehrere Tenside, ausgewählt aus Phenolat-Tensiden, Salicylat-Tensiden und Sulfonat-Tensiden, wobei das eine oder die mehreren Tenside jeweils unabhängig einen TBN-Wert (total base number; basischer Gesamtwert) im Bereich von 30 bis 350 mg.KOH/g, gemessen nach ISO 3771, aufweisen; und
(B) zumindest 3,5 Gew.-% von einem oder mehreren Antioxidantien, basierend auf dem Gesamtgewicht der Schmierölzusammensetzung, wobei das eine oder die mehreren Antioxidantien in der Schmierölzusammensetzung aminische Antioxidantien umfassen.

2. Verwendung nach Anspruch 1, wobei das eine oder die mehreren Antioxidantien in der Schmierölzusammensetzung in einer Menge von zumindest 3,7 Gew.-% vorhanden sind, basierend auf dem Gesamtgewicht der Schmierölzusammensetzung.

3. Verwendung nach Anspruch 1 oder 2, wobei das eine oder die mehreren aminischen Antioxidantien aus alkylierten Diphenylaminen, Phenyl-α-naphthylaminen, Phenyl-β-naphthylaminen und alkylierten α-Naphthylaminen ausgewählt sind.

4. Verwendung nach einem der Ansprüche 1 bis 3, wobei die Schmierölzusammensetzung einen Schwefelgehalt von nicht größer als 1,2 Gew.-%, basierend auf dem Gesamtgewicht der Schmierölzusammensetzung, aufweist.

5. Verwendung nach einem der Ansprüche 1 bis 4, wobei die Schmierölzusammensetzung einen Phosphorgehalt im Bereich von 0,04 bis 0,09 Gew.-%, basierend auf dem Gesamtgewicht der Schmierölzusammensetzung, aufweist.

6. Verwendung nach einem der Ansprüche 1 bis 5, wobei der TBN-Wert einer frischen, unbenutzten Probe der Schmierölzusammensetzung im Bereich von 5,0 bis 12,0 mg.KOH/g, gemessen nach ISO 3771, liegt.

7. Verwendung nach einem der Ansprüche 1 bis 6, wobei die Veränderung des TBN-Wertes einer frischen, unbenutzten Probe der Schmierölzusammensetzung, gemessen nach ISO 3771, und der TBN-Wert bei Testende (VW-T4-Test (PV 1449)) derselben Schmierölzusammensetzung, gemessen nach ISO 3771, kleiner als 2,5 mg.KOH/g ist.

## Revendications

1. Utilisation d'une composition d'huile de lubrification pour maintenir un niveau de TBN d'au moins 5,0 mg.KOH/g, tel que mesuré par la norme ISO 3771, dans un moteur à combustion interne dans le test VW T4 (PV 1449) dans lequel la composition d'une huile de lubrification a un contenu en cendres sulfatées qui n'est pas plus grand que 0,9 % en poids et un contenu en phosphore dans la plage allant de 0,04 à 0,1 % en poids, et la composition d'huile de lubrification comprend une huile de base,
(A) un ou plusieurs détergents sélectionnés à partir de détergents de type phénate, de détergents de type salicylate et de détergents de type sulfonate, dans lesquels les un ou plusieurs détergents ont chacun, de manière indépendante, une valeur de TBN (nombre de base total) dans la plage allant de 30 à 350 mg.KOH/g, telle que mesurée par la norme ISO 3771 ; et
(B) au moins 3,5 % en poids d'un ou plusieurs antioxydants, sur la base du poids total de la composition d'huile de lubrification, les un ou plusieurs antioxydants dans la composition d'huile de lubrification comprenant des antioxydants de type amine.

2. Utilisation selon la revendication 1, dans laquelle les un ou plusieurs antioxydants sont présents dans la composition d'huile de lubrification dans une quantité d'au moins 3,7 % en poids, sur la base du poids total de la composition d'huile de lubrification.

3. Utilisation selon la revendication 1 ou 2, dans laquelle les un ou plusieurs antioxydants de type amine sont sélectionnés à partir de diphénylamines alkylatées, de phényl-α-naphtylamines, de phényl-α-naphtylamines et de α-naphtylamines alkylatées.

4. Utilisation selon l'une quelconque des revendications 1 à 3, dans laquelle la composition d'huile de lubrification a une teneur en soufre qui n'est pas plus grande que 1,2 % en poids, sur la base du poids total de la composition d'huile de lubrification.

5. Utilisation selon l'une quelconque des revendications 1 à 4, dans laquelle la composition d'huile de lubrification a une teneur en phosphore dans la plage allant de 0,04 à 0,09 % en poids, sur la base du poids total de la composition d'huile de lubrification.

6. Utilisation selon l'une quelconque des revendications 1 à 5, dans laquelle la valeur de TBN d'un échantillon inutilisé neuf de la composition d'huile de lubrification est dans la plage allant de 5,0 à 12,0 mg.KOH/g, telle que mesurée par la norme ISO 3771.

7. Utilisation selon l'une quelconque des revendications 1 à 6, dans laquelle le changement de la valeur de TBN d'un échantillon inutilisé neuf de la composition d'huile de lubrification telle que mesurée par la norme ISO 3771, et la valeur de TBN de fin de test (VW T4 Test (PV 1449)) de la même composition d'huile de lubrification, telle que mesurée par la norme ISO 3771, est inférieur à 2,5 mg.KOH/g.
